

## UNITED STATES PATENT OFFICE

2,446,468

## SELENIUM RECTIFIERS

Stanley S. Fry, North Chicago, Ill., assignor to  
 Fansteel Metallurgical Corporation, North Chicago, Ill., a corporation of New York

No Drawing. Application June 14, 1945.  
 Serial No. 599,518

13 Claims. (Cl. 175—366)

1

This invention relates to selenium rectifiers. In the production of selenium rectifiers, a rigid carrier electrode or supporting electrode is provided with a thin coating or layer of selenium. The supporting electrode may be formed of nickel, nickel-plated iron, aluminum, magnesium, beryllium or other metals and alloys. A common practice in the production of selenium rectifiers includes grit blasting the iron disc or plate and electroplating the disc with nickel. The purpose of the grit blasting is to present a roughened surface to the selenium and to thereby improve the adherence of the selenium to the carrier electrode. The disc is then thoroughly cleaned and a thin film of selenium is applied over the nickel layer.

The selenium film or layer may be formed by a variety of methods. The plate or disc may be heated to a temperature above the melting point of selenium, for example, to a temperature of from 230° C. to 250° C., and the selenium in stick form may be rubbed across the heated plate in order to melt the selenium and form the desired film. Another method of application includes placing a measured quantity of powdered selenium or selenium in pellet form on the heated plate and flowing the melted selenium over the surface. The melted selenium is usually spread over the heated plate by mechanical means, as with a glass rod. The selenium may also be deposited on the carrier electrode from a vapor phase. The vaporization method is commonly employed in depositing the selenium film upon the light metal carrier electrodes. Various materials may be added to the selenium to increase its conductivity and otherwise impart desired characteristics and properties.

The selenium is then transformed into its gray, crystalline state by heat treatment. The coated discs are generally stacked with mica, aluminum or other inert, smooth-surfaced discs or washers in contact with the selenium and between adjacent plates, and the stack subjected to a moderate pressure. The stacks under pressure are then subjected to a relatively low temperature, that is, a temperature below 150° C., and maintained at such temperature for from one hour to four or five hours. During this stage of the heat treatment the selenium softens so that the pressure produces a layer of selenium of relatively uniform thickness and having a smooth surface.

The stacks are withdrawn from the oven or heat treating furnace and the plates are removed from the stack. The plates are then given a further heat treatment at a temperature approach-

2

ing the melting point of selenium. This heat treatment is generally conducted at temperatures between about 200° C. and the melting point of selenium, for example, about 210° C., for a period of from fifteen minutes to several hours. During the combined heat treatment, a layer of selenium is produced having a smooth surface of more or less uniform thickness and the selenium is transformed from its amorphous, non-conducting form into its gray, crystalline, conducting form.

The smooth surface of the selenium film is then treated to form an artificial blocking layer and a counter-electrode consisting of a relatively low melting point alloy is applied, as by spraying, over the selenium coating.

The final step in the manufacture of the rectifier plates consists of an electrical forming treatment. This treatment consists of subjecting the plate to either an alternating or direct current until a high resistance is developed in the reverse direction. This step may consist of applying to the plate in the reverse direction a direct current voltage below about 15 volts or a pulsating direct current starting with a low voltage of about 8 volts and gradually increasing the voltage to about 21 volts over a period of several hours.

In the use of an alternating current, it is necessary to include in the circuit a current limiting resistor because one-half cycle flows in the forward direction of the rectifier plate. The voltage may be about 20 volts and the period required for forming is generally greater than that required when a direct current is employed because only one-half cycle of the current flows in the reverse direction.

Light sensitive devices of the blocking layer class are produced in a similar manner. A supporting electrode is provided with a thin film or layer of selenium in its gray, crystalline modification and an artificial blocking layer formed on the surface of the selenium. A second electrode is then applied over the treated surface of the selenium. This electrode may consist of a light-permeable film of metal or a metal grid. The application of the light-permeable metal may be accomplished by any of the methods known to the art.

This invention is directed to the manufacture of selenium rectifiers provided with a specific type of counter-electrode. The method is not limited to any specific form, type or composition of carrier electrode. Any method may be employed in providing the carrier electrode with the film or layer of gray, crystalline, conducting selenium. The selenium layer may or may not contain added

materials to impart desired characteristics and properties. An artificial blocking layer may be formed on the surface of the selenium in any desired manner.

The principal object of this invention is to provide a counter-electrode of novel composition.

A further object of this invention is to provide a selenium rectifier element having an appreciably higher break down voltage than selenium rectifiers made with the usual and conventional low melting point counter-electrode.

Other objects and advantages of this invention will become apparent from the following description and claims.

In conventional methods of production of selenium rectifier elements, the counter-electrode consists of a low melting point alloy of bismuth, cadmium and tin. The particular composition of the alloy differs with various manufacturers depending in most instances upon individual preference. Commonly, the alloy consists of 45% to 55% bismuth, 20 to 30% tin and 20 to 25% cadmium, a common alloy containing 54% bismuth, 26% tin and 20% cadmium. This alloy has a melting point of about 130° C. Another common alloy consists of Wood's metal, contains approximately 50% bismuth, 25% lead, 12.5% cadmium and 12.5% tin and has a melting point of about 65.5° C. Various tin-cadmium alloys and bismuth-cadmium alloys have been proposed. For example, in Patent No. 2,235,051 there is disclosed tin-cadmium alloys containing 25% to 60% cadmium. An alloy of 68% tin and 32% cadmium has a melting point of about 180° C. The counter-electrode disclosed in Patent No. 2,193,610 consists of 75% tin and 25% cadmium and has a melting point of about 165° C.

Selenium rectifiers provided with counter-electrodes of these alloys are generally operated at an applied alternating current voltage of about 14 to 18 volts since the rectifier elements break down at voltages in excess of about 18 volts when applied continuously. In some instances this voltage limitation has been a disadvantage in the use of selenium rectifiers.

I have discovered that the addition of small amounts of magnesium to the counter-electrode alloy greatly increases the voltage which may be safely and continuously applied to the selenium rectifier. The amount of magnesium does not appear to be particularly critical so far as the operation of the selenium rectifiers is concerned. The principal limitation is the production of a low melting point alloy. For these purposes I have found that alloys containing magnesium in amounts up to about 2%, preferably from about 0.25% to about 2%, are generally the most satisfactory. Alloys containing higher amounts are satisfactory; however, they do present difficulties in melting and spraying of the alloy upon the selenium layer. In some instances, I have found that it is advantageous to provide a counter-electrode in the form of an exceedingly thin sprayed coating containing magnesium and coating or covering this thin film with the usual counter-electrode containing no magnesium so as to provide a better mechanical layer or film.

Selenium rectifiers provided with a magnesium containing counter-electrode may be operated at applied alternating current voltages between 30 and 35 volts without danger of breakdown.

The production of the selenium rectifiers may be identical to that commonly used wherein a

carrier electrode is provided with a thin film or layer of selenium in its gray, crystalline modification. An artificial blocking layer may be provided by any desired manner. The counter-electrode of this invention is applied as by spraying according to well known practice. The final step is the electrical forming process which is also known to the art.

One of the methods commonly employed in grading and in evaluating the quality of selenium rectifier plates is the measurement of the current passed by the plate in the reverse or blocking direction upon application of a direct current voltage to the plate in the blocking direction. An ideal or theoretically perfect rectifier plate would have no leakage current flow under such condition.

In order to compare the current leakage of rectifier plates made in accordance with the present invention and of rectifier plates made with a conventional counter-electrode, a group of nickel-plated iron discs, each having an area of approximately 3 sq. cm., was provided with a layer of selenium in its gray, crystalline form. The discs were heated to a temperature of about 240° C. and selenium in stick form rubbed across the plate. The selenium was spread over the surface of the heated discs with a glass rod. The plates were then stacked with mica discs covering the selenium layer and the stack placed under pressure. The stack was heated to a temperature below 150° C. for about 2 hours. The pressure was then removed and the plates heated to about 210° C. and maintained at this temperature for about 1/2 hour.

The group of plates was then divided into two series. The first series of plates was provided with a counter-electrode consisting of approximately 54% bismuth, 26% tin and 20% cadmium. The second series of plates was provided with a counter-electrode consisting of the same alloy to which had been added about 2% magnesium. The discs of the series of plates provided with the counter-electrode of the invention were subjected to an electrical forming treatment by the application of a rectified alternating current voltage to each plate in the reverse or blocking direction, the rectified voltage reaching a maximum of about 34 volts. The discs or plates provided with the conventional counter-electrode were subjected to an electrical forming treatment by the application of a rectified alternating current voltage to each plate in the reverse or blocking direction, the rectified voltage reaching a maximum of about 21 volts. It is not possible to apply a voltage much greater than 21 volts to these plates because the counter-electrodes melt and destroy the rectifier upon the application of voltages between about 23 volts and 25 volts.

A direct current voltage of 34 volts from a storage battery source was applied in the reverse or blocking direction to the individual discs of each series. The leakage current or the reverse current flowing in the standard plates averaged approximately 25 milliamperes. The leakage current in the plates provided with the counter-electrode of this invention averaged approximately 2 milliamperes. In the case of the standard or control plates it was necessary to measure or read the current flow as rapidly as possible because at this applied voltage the counter-electrode melts in a short period which may be less than one minute. In the case of the plates having a counter-electrode of this in-

vention, the continuous application of this voltage does not damage or injure the rectifier and such plates may be operated at applied alternating current voltages up to 34 or 35 volts.

The improvements in the operating characteristics of rectifier plates made in accordance with this invention are quite apparent from this data. It is obvious that the numerical values of the leakage current will differ with different size rectifier plates and also with selenium having various addition agents. The data, however, is representative of the improvements attained in the practice of my invention. The improvements obtained by the addition of small amounts of magnesium are not limited to the specific bismuth-tin-cadmium alloys set forth in the specific example but are also obtained when magnesium is added to other bismuth-tin-cadmium alloys and other low melting point alloys of the type commonly used in providing selenium rectifier elements with counter-electrodes.

I claim:

1. A blocking layer device comprising a carrier electrode, a layer of gray, crystalline selenium and a counter-electrode consisting essentially of bismuth, tin, lead, cadmium and a small amount of magnesium, the counter-electrode having a melting point not exceeding 180° C.

2. A blocking layer device comprising a carrier electrode, a layer of gray, crystalline selenium and a counter-electrode consisting essentially of bismuth, tin, lead, cadmium and from about 0.25% to about 2% magnesium, the counter-electrode having a melting point not exceeding 180° C.

3. A selenium rectifier comprising a carrier electrode, a layer of gray, crystalline selenium and a counter-electrode consisting essentially of bismuth, tin, lead, cadmium and a small amount of magnesium, the counter-electrode having a melting point not exceeding 180° C.

4. A selenium rectifier comprising a carrier electrode, a layer of gray, crystalline selenium and a counter-electrode consisting essentially of bismuth, tin, lead, cadmium and from about 0.25% to about 2% magnesium, the counter-electrode having a melting point not exceeding 180° C.

5. A selenium rectifier comprising a carrier electrode, a layer of gray, crystalline selenium and a counter-electrode consisting essentially of bismuth, tin, cadmium and a small amount of magnesium.

6. A selenium rectifier comprising a carrier electrode, a layer of gray, crystalline selenium and a counter-electrode consisting essentially of bismuth, tin, cadmium and from about 0.25% to about 2% magnesium.

7. A selenium rectifier comprising a carrier electrode, a layer of gray, crystalline selenium and a counter-electrode composed of an alloy consist-

ing of about 45% to about 55% bismuth, about 20% to about 30% tin, about 20% to about 25% cadmium and magnesium in amounts up to about 2%.

5 8. A selenium rectifier comprising a carrier-electrode, a layer of gray, crystalline selenium and a counter-electrode composed of an alloy consisting essentially of bismuth, cadmium and magnesium in amounts up to about 2%.

10 9. A selenium rectifier comprising a carrier electrode, a layer of gray, crystalline selenium on the carrier electrode, a thin layer of an alloy of bismuth, tin, cadmium and magnesium on the selenium layer and a layer of an alloy of bismuth, tin and cadmium on the first named alloy layer.

15 10. A selenium rectifier comprising a carrier electrode, a layer of gray, crystalline selenium, a thin layer of an alloy consisting essentially of bismuth and cadmium and containing magnesium on the selenium layer and an exterior layer of an alloy consisting essentially of bismuth and cadmium.

11. A selenium rectifier comprising a carrier electrode, a layer of gray, crystalline selenium and a counter-electrode, the counter-electrode comprising a thin layer of an alloy on the selenium layer, the alloy consisting essentially of bismuth, tin, lead, cadmium and a small amount of mag-

25 nesium and having a melting point not exceeding 180° C., and an exterior layer of an alloy over the magnesium containing layer, the last named alloy consisting essentially of bismuth, tin, lead and cadmium and having a melting point not exceeding 180° C.

30 35 12. A selenium rectifier comprising a carrier electrode, a layer of gray, crystalline selenium and a counter-electrode composed of an alloy consisting essentially of cadmium, tin and magnesium in amounts up to about 2%.

40 45 13. A selenium rectifier comprising a carrier electrode, a layer of gray, crystalline selenium, a thin layer of an alloy consisting essentially of cadmium and tin and containing magnesium on the selenium layer and an exterior layer of an alloy consisting essentially of cadmium and tin.

STANLEY S. FRY.

#### REFERENCES CITED

The following references are of record in the 50 file of this patent:

#### UNITED STATES PATENTS

| Number    | Name               | Date          |
|-----------|--------------------|---------------|
| 1,826,955 | Ruben et al. ----- | Oct. 13, 1931 |
| 1,866,351 | Hollnagel -----    | July 5, 1932  |
| 2,039,083 | Keiffer -----      | Apr. 28, 1936 |
| 2,162,487 | Lotz -----         | June 13, 1939 |
| 2,175,016 | Brunke -----       | Oct. 3, 1939  |
| 2,221,596 | Lorenz -----       | Nov. 12, 1940 |